

## UNITED STATES PATENT OFFICE

CHARLES F. RUDZENIA, OF OAKLAND, CALIFORNIA

## CLEANING FLUID

No Drawing.

Application filed March 1, 1927. Serial No. 171,912.

My invention relates to an improved cleaning fluid consisting of saponified oils and fatty acid, acetone, vegetable oils, and hydrocarbon solvents mixed to constitute a new 5 composition of matter.

The primary object of my invention is to provide, as a new composition of matter, an improved cleaning fluid.

Another object is to provide an improved 10 composition which may be used economically and efficiently by dry cleaners and the like, for removing dirt and spots of various natures from fabrics of substantially all kinds without injury to the fabric.

15 A further object is to provide a new and improved composition which can be manufactured economically.

My improved composition of matter consists broadly of a fluid mixture of saponified 20 fatty acid and vegetable oils, water, acetone, and hydrocarbon solvents. More specifically, my improved composition consists of the following ingredients mixed in substantially the portions given:

|                       | Per cent |
|-----------------------|----------|
| 25 Fatty acid (oleic) | 33       |
| Pine oil              | 15       |
| Potash                | 5        |
| Water                 | 10       |
| 30 Petrolatum (soft)  | 5        |
| Benzene               | 4.50     |
| Alcohol               | 1.25     |
| Acetone               | 12.50    |
| Banana oil            | 0.50     |
| 35 Cocoanut oil       | 0.75     |
| Hydrocarbon solvent   | 12.50    |

In mixing the above ingredients to produce my new composition of matter, the fatty acid, preferably oleic acid, and potash are first 40 mixed and brought to boiling. To the heated mixture water and pine oil is added in substantially the proportions above given, the entire mixture being agitated and thoroughly mixed. The remaining ingredients 45 are then mixed together and added and mixed with the saponified fatty acid after the saponified mixture has been allowed to cool.

The hydrocarbon solvent above mentioned 50 may be of various kinds. Gasoline or other petroleum distillation product of relatively

low specific gravity may be used for the purpose.

The above mixture constitutes a highly efficient cleaning fluid for removing spots from clothing and the like and for dry 55 cleaning fabrics of substantially all kinds. As an agent for dry cleaning, the mixture is used in the dry cleaning process in the same manner, and as a substitute for gasoline. The combined action of the several active ingredients of my mixture renders the mixture 60 highly efficient in removing dirt and spots of various natures in the single cleaning process, thereby avoiding much of the time and labor commonly required for removing spots and dirt not effected by the gasoline or removed during the regular 65 cleaning operation.

While I have given the specific ingredients and proportioning which I prefer, the mixture may, of course, be modified within reasonable limits without departing from the spirit of the invention. I, therefore, do not wish to restrict myself to the exact ingredients and the specific proportions stated, but 70 desire to avail myself of any variation which may fall within the scope of the appended claim.

Having thus described my invention what I claim as new and desire to secure by Letters 80 Patent, is:

As a composition of matter, a cleaning fluid formed by mixing the following ingredients in the following proportions: fatty acids 33%; pine oil 15%; potash 5%; water 10%; soft petrolatum 5%; benzene 41/2%; alcohol 1 1/4%; acetone 12 1/2%; banana oil 1/2%; cocoanut oil 3/4%; and hydrocarbon solvent 12 1/2%.

In witness whereof I hereunto set my 90 signature.

CHARLES F. RUDZENIA.

95